

## 1

2,989,490

### ELECTRICAL CONTACT BRUSH FOR HIGH ALTITUDE USE

Dimitar Ramadanoff, Berea, Ohio, assignor to Union Carbide Corporation, a corporation of New York  
No Drawing. Filed Feb. 19, 1958, Ser. No. 716,009  
13 Claims. (Cl. 252—503)

This invention relates to brushes for the supply of electric current, and more particularly concerns long wearing commutator brushes which are suitable for use at conditions encountered at both sea level and at high altitudes.

For sea level and high altitude applications, metal graphite brushes, such as high altitude copper-graphite brushes, have several desirable properties. At a given current density and rubbing speed, the copper-graphite brushes generally operate with a lower contact voltage drop and a lower temperature at a given load than do high altitude electrographitic brushes. The brush stock has low electrical resistivity, which is helpful in cutting down power losses. But copper-graphite brushes also have some disadvantages. They operate with higher coefficients of friction than electrographitic brushes, and are sensitive to commutator or ring eccentricity. Sometimes the combination of these two factors may intensify sparking, and even cause, under some conditions, the release of small streamers at the trailing edges which may lead to undesirable ring wear. Consequently, the conventional copper-graphite brushes are usually limited in their application.

It is, therefore, an important object of the present invention to provide an improved metal graphite brush composition which is not subject to this difficulty, either under atmospheric or high altitude operation.

Another object of the present invention is to provide an improved metal graphite brush suitable for use at varying altitudes, which will deposit a boundary lubricating film upon the commutator surface at both high and low altitudes, and which will not unduly wear the commutator during the life of the brush.

The conventional metal graphite brush containing approximately 25% to 75% copper, 10% to 60% graphite, a small amount of binder material and 5% to 25% of a compound selected from the group consisting of barium fluoride, strontium carbonate and calcium carbonate has some unusually good properties as a high altitude brush, for example, a brush of the above noted type having a composition of about 75 percent copper, 15 percent graphite and 10 percent barium fluoride has an electrical resistivity of 0.000008 ohm per cubic inch. Its contact voltage drop of 0.35 volt with a current density of 180 amperes per square inch at an altitude of 40,000 feet above sea level is one of the lowest on record. Such a brush grade has proven to commute very well, and due to its barium fluoride content, has resisted dusting at altitudes up to 70,000 feet. A weakness possessed by this copper graphite brush which is representative of the behavior of brushes falling within the above composition range is its short life under some conditions. It has an average brush life of only 825 hours per inch at sea level, and 425 hours per inch under simulated altitude conditions at 40,000 feet.

According to the present invention, it has been found that the life of a conventional metal-graphite sliding contacting element operating in atmospheres such as exist at sea level and at altitudes of at least 40,000 feet can be greatly lengthened and contact conditions materially improved if the brush composition is made from certain materials.

A brush embodying my invention is a metal-graphite

## 2

composition composed of 25 percent to 75 percent copper, 10 percent to 60 percent graphite and 5 percent to 25 percent of at least one compound selected from the group consisting of barium fluoride, strontium carbonate and calcium carbonate, 0.1% to 5% boron nitride, and up to 10% in the aggregate of silver or lead or tin or mixtures thereof. Coumarone indene resin may also be incorporated in the brush of the invention with or without the presence of the enumerated metals in a proportion of up to 5%. Generally, the sum of boron nitride, metal and resin used in the brush composition should be between 0.1 percent and 15.0 percent by weight of the brush. A preferred range for boron nitride is 0.5% to 1.5%. If the metals are present, a preferred range for the aggregate is 4% to 6%. Also, if the resin is present, the preferred range is 2% to 3%, all percentages being by weight of the brush.

The invention will be more fully understood from the following detailed description of typical examples of its use for prolonging brush life at sea level or high altitude conditions, it being understood that these examples are presented as illustrative only, and that they are not intended to limit the scope of the invention.

### EXAMPLE I

25 The composition of a copper-graphite mixture containing 75 parts copper, 15 parts graphite, 10 parts barium fluoride and a small amount of binder material was modified by adding to it 1 part boron nitride powder. The said 30 ingredients were then well mixed and molded at a pressure of 15 tons per square inch to a block of suitable size for making a commutator brush. The block was then baked at 900° C. by suitable heating means for a period sufficient to impart known and inherent brush 35 characteristics.

### EXAMPLE II

To a mixture having the composition of Example I containing 1 part boron nitride, was added 5 parts metallic silver powder. The mixture was formed into the shape 40 of a commutator brush, and baked in the manner described in Example I to impart to it the requisite brush characteristics.

### EXAMPLE III

45 To a mixture having the composition of Example II containing 1 part boron nitride and 5 parts silver, there was added about 2.5 parts coumarone indene resin. The mixture was then formed and baked in the manner previously described.

The three additive compounds, whose performance it is sought to improve, are similar in a number of respects. Strontium carbonate, barium fluoride and calcium carbonate are all insoluble, non-deliquescent salts of alkaline earth metals. When added to a copper-graphite brush, the brush containing each salt has good friction properties and a minimum of sliding wear on the bearing surface.

Brushes embodying the invention have been made and tested at sea level and under conditions simulating altitudes up to 60,000 feet above sea level. All tests were 50 conducted by applying the brush to a machine having an operating speed of 6500 revolutions per minute and a rubbing speed of 5100 feet per minute. A brush spring pressure of 7.1 pounds per square inch was used. The current flow through the brush was adjusted to 20 or 40 amperes or a current density of about 60 or 120 amperes per square inch depending upon the altitude. Tests were 55 conducted in room air for a total of 20 hours or more. During that time readings were taken of contact voltage drop, brush temperature, and coefficient of friction. At 60 the end of the tests brush length was measured and brush life in hours per inch of wear was calculated. All altitude tests were made on rotating copper rings.

In similar fashion, a number of other brushes were tested, the compositions, operating conditions and properties being shown in Table I which sets forth the conditions and results of a number of typical tests wherein the brush was tested at sea level conditions, and at an altitude of 40,000 feet. In these tests the brushes were subjected to current densities of 60 and 120 amperes per square inch at sea level, and current densities of 60 and 120 amperes per square inch at 40,000 feet altitude.

Table I

| Brush          | Composition by weight percent |      |                  |                   |                   |    |    |    |    |       |
|----------------|-------------------------------|------|------------------|-------------------|-------------------|----|----|----|----|-------|
|                | Cu                            | C    | BaF <sub>2</sub> | SrCO <sub>3</sub> | CaCO <sub>3</sub> | BN | Ag | Pb | Sn | Resin |
| A <sup>1</sup> | 75                            | 15   | 10               | 0                 | 0                 | 0  | 0  | 0  | 0  | 0     |
| B              | 74                            | 15   | 10               | 0                 | 0                 | 1  | 0  | 0  | 0  | 0     |
| C              | 69                            | 15   | 10               | 0                 | 0                 | 1  | 5  | 0  | 0  | 0     |
| D              | 68                            | 14   | 9.5              | 0                 | 0                 | 1  | 5  | 0  | 0  | 2.5   |
| E <sup>1</sup> | 45                            | 45   | 10               | 0                 | 0                 | 0  | 0  | 0  | 0  | 0     |
| F              | 45                            | 45   | 9                | 0                 | 0                 | 1  | 0  | 0  | 0  | 0     |
| G              | 42                            | 42   | 10               | 0                 | 0                 | 1  | 5  | 0  | 0  | 0     |
| H              | 42                            | 42   | 10               | 0                 | 0                 | 1  | 0  | 5  | 0  | 0     |
| I              | 42                            | 42   | 10               | 0                 | 0                 | 1  | 0  | 0  | 5  | 0     |
| J <sup>1</sup> | 47.5                          | 47.5 | 0                | 5                 | 0                 | 0  | 0  | 0  | 0  | 0     |
| K              | 47                            | 47   | 0                | 5                 | 0                 | 1  | 0  | 0  | 0  | 0     |
| L              | 44.5                          | 44.5 | 0                | 5                 | 0                 | 1  | 5  | 0  | 0  | 0     |
| M              | 44.5                          | 44.5 | 0                | 5                 | 0                 | 1  | 0  | 5  | 0  | 0     |
| N              | 44.5                          | 44.5 | 0                | 5                 | 0                 | 1  | 0  | 5  | 0  | 0     |
| O <sup>1</sup> | 47.5                          | 47.5 | 0                | 0                 | 5                 | 0  | 0  | 0  | 0  | 0     |
| P              | 47                            | 47   | 0                | 0                 | 5                 | 1  | 0  | 0  | 0  | 0     |
| Q              | 44.5                          | 44.5 | 0                | 0                 | 5                 | 1  | 5  | 0  | 0  | 0     |

<sup>1</sup> Conventional high altitude brush composition.

| Brush          | Operating Properties |                                    |                     |                  |                                        |                                  |
|----------------|----------------------|------------------------------------|---------------------|------------------|----------------------------------------|----------------------------------|
|                | Altitude             | Current Density, Amps. Per Sq. Ft. | Contact Drop, Volts | Brush Temp., °C. | Brush Life, <sup>2</sup> Hrs. Per Inch | Coef. of Friction Against Copper |
| A <sup>1</sup> | 0                    | 60                                 | .14                 | 95               | 895                                    | <sup>3</sup> NT                  |
|                | 40,000               | 120                                | .24                 | 70               | 425                                    | .10                              |
| B              | 0                    | 60                                 | .17                 | 92               | 1,455                                  | NT                               |
|                | 40,000               | 120                                | .32                 | 72               | 745                                    | .10                              |
| C              | 0                    | 60                                 | .13                 | 98               | 1,170                                  | NT                               |
|                | 40,000               | 120                                | .38                 | 70               | 1,000                                  | .103                             |
| D              | 0                    | 60                                 | .23                 | 88               | 2,365                                  | NT                               |
|                | 40,000               | 120                                | .44                 | 68               | 940                                    | .07                              |
| E <sup>1</sup> | 0                    | 60                                 | .53                 | 114              | 6,800                                  | NT                               |
|                | 40,000               | 60                                 | .23                 | 170              | 760                                    | .35                              |
| F              | 0                    | 60                                 | 1.0                 | 130              | 4,300                                  | NT                               |
|                | 40,000               | 60                                 | .55                 | 146              | 4,300                                  | .195                             |
| G              | 0                    | 60                                 | .45                 | 126              | 6,590                                  | NT                               |
|                | 40,000               | 120                                | .88                 | 120              | 3,450                                  | .125                             |
| H              | 0                    | 120                                | 1.29                | 138              | 5,200                                  | .14                              |
|                | 40,000               | 120                                | 1.20                | 206              | 1,900                                  | .16                              |
| I              | 0                    | 60                                 | .56                 | 121              | 9,800                                  | NT                               |
|                | 40,000               | 60                                 | .65                 | 166              | 880                                    | .196                             |
| J <sup>1</sup> | 0                    | 120                                | 1.04                | 120              | 6,300                                  | .18                              |
|                | 40,000               | 60                                 | .25                 | 87               | 858                                    | .19                              |
| K              | 0                    | 120                                | .94                 | 103              | 8,850                                  | .14                              |
|                | 40,000               | 60                                 | .39                 | 108              | 1,688                                  | .184                             |
| L              | 0                    | 120                                | .92                 | 88               | 11,548                                 | .09                              |
|                | 40,000               | 60                                 | .29                 | 110              | 1,070                                  | .178                             |
| M              | 0                    | 120                                | 1.07                | 131              | 11,760                                 | .16                              |
|                | 40,000               | 60                                 | .42                 | 152              | 1,000                                  | .161                             |
| N              | 0                    | 120                                | .65                 | 112              | 14,035                                 | .10                              |
|                | 40,000               | 60                                 | .43                 | 112              | 1,565                                  | .170                             |
| O <sup>1</sup> | 0                    | 120                                | .36                 | 151              | 3,050                                  | .26                              |
|                | 40,000               | 60                                 | .48                 | 140              | 1,000                                  | .18                              |
| P              | 0                    | 120                                | .73                 | 120              | 5,230                                  | .144                             |
|                | 40,000               | 60                                 | .60                 | 95               | 1,000                                  | .139                             |
| Q              | 0                    | 120                                | 1.00                | 114              | 5,100                                  | .133                             |
|                | 40,000               | 60                                 | .75                 | 78               | 1,140                                  | .118                             |

<sup>1</sup> Conventional brush composition.

<sup>2</sup> The life measurement is an average obtained for altitudes from 20,000 feet to 60,000 feet. The time at 40,000 feet is predominating.

<sup>3</sup> Not tested.

From the data in Table I it will be seen that for a high altitude brush of the copper graphite type, herein disclosed, better performance can be obtained at sea level and under altitude conditions if the brush contains as additive material, predetermined quantities of either boron nitride alone or in combination with one or more members in the group consisting of silver, lead, tin, and coumarone indene resin. The improved performance manifests itself in relatively long brush life, small ring wear, generally lower coefficient of friction, low operating tem-

peratures, high current load capacity and higher operating altitudes.

This application is a continuation-in-part of application Serial No. 493,070, filed March 8, 1955, now abandoned.

5 What is claimed is:

1. An electrical contact brush adapted to operate efficiently at altitudes of at least 40,000 feet consisting of 25% to 75% copper, 10% to 60% graphite, 0.1% to 5% boron nitride, 5% to 25% in the aggregate of at least one compound selected from the group consisting of barium fluoride, strontium carbonate and calcium carbonate, up to 5% coumarone indene resin and up to 10% in the aggregate of at least one metal selected from the group consisting of lead, silver and tin.

15 2. An electrical contact brush adapted to operate efficiently at altitudes of at least 40,000 feet consisting of 25% to 75% copper, 10% to 60% graphite, 5% to 25% of at least one compound selected from the group consisting of strontium carbonate, calcium carbonate and barium fluoride and 0.1% to 5% boron nitride.

20 3. An electrical contact brush adapted to operate efficiently at altitudes of at least 40,000 feet consisting of 25% to 75% copper, 10% to 60% graphite, 5% to 25% of at least one compound selected from the group consisting of strontium carbonate, calcium carbonate and barium fluoride, 0.1% to 5% boron nitride and 1% to 10% in the aggregate of at least one metal selected from the group consisting of silver, lead and tin.

30 4. An electrical contact brush adapted to operate efficiently at altitudes of at least 40,000 feet consisting of 25% to 75% copper, 10% to 60% graphite, 5% to 25% of at least one compound selected from the group consisting of strontium carbonate, calcium carbonate and barium fluoride, 0.1% to 5% boron nitride, 1% to 10% in the aggregate of at least one metal selected from the group consisting of silver, lead and tin, and 1% to 5% coumarone indene resin.

35 5. An electrical contact brush adapted to operate efficiently at altitudes of at least 40,000 feet consisting of 25% to 75% copper, 10% to 60% graphite, 5% to 25% of at least one compound selected from the group consisting of strontium carbonate, calcium carbonate and barium fluoride, 0.1% to 5% boron nitride and 1% to 5% coumarone indene resin.

40 6. An electrical contact brush adapted to operate efficiently at altitudes of at least 40,000 feet consisting of 25% to 75% copper, 10% to 60% graphite, 5% to 25% of a compound selected from the group consisting of strontium carbonate, calcium carbonate and barium fluoride, and additive material consisting of 0.1% to 5% boron nitride, up to 5% coumarone indene resin and up to 10% in the aggregate of at least one metal selected from the group consisting of lead, silver and tin, said additive material comprising 0.1% to 15% by weight of said brush.

45 7. An electrical contact brush adapted to operate efficiently at altitudes of at least 40,000 feet consisting of 25% to 75% copper, 10% to 60% graphite, 5% to 25% of a compound selected from the group consisting of strontium carbonate, calcium carbonate and barium fluoride, and additive material consisting of 0.1% to 5% boron nitride, up to 5% coumarone indene resin and up to 10% in the aggregate of at least one metal selected from the group consisting of lead, silver and tin, and silver.

50 8. An electrical contact brush adapted to operate efficiently at altitudes of at least 40,000 feet consisting of 25% to 75% copper, 10% to 60% graphite, 5% to 25% barium fluoride, 0.1% to 5% boron nitride, up to 5% coumarone indene resin and up to 10% of at least one metal selected from the group consisting of lead, tin, and silver.

55 9. An electrical contact brush adapted to operate efficiently at altitudes of at least 40,000 feet consisting of 25% to 75% copper, 10% to 60% graphite, 5% to 25% barium fluoride and 0.1% to 5% boron nitride.

60 10. An electrical contact brush adapted to operate efficiently at altitudes of at least 40,000 feet consisting of 25% to 75% copper, 10% to 60% graphite, 5% to 25% barium fluoride and 0.1% to 5% boron nitride and 10% silver.

65 11. An electrical contact brush adapted to operate efficiently at altitudes of at least 40,000 feet consisting of 25% to 75% copper, 10% to 60% graphite, 5% to 25% barium fluoride and 0.1% to 5% boron nitride.

70 12. An electrical contact brush adapted to operate efficiently at altitudes of at least 40,000 feet consisting of 25% to 75% copper, 10% to 60% graphite, 5% to 25% barium fluoride, 0.1% to 5% boron nitride and 1% to 10% silver.

75 13. An electrical contact brush adapted to operate efficiently at altitudes of at least 40,000 feet consisting of 25% to 75% copper, 10% to 60% graphite, 5% to 25%

barium fluoride, 0.1% to 5% boron nitride and 1% to 10% lead.

11. An electrical contact brush adapted to operate efficiently at altitudes of at least 40,000 feet consisting of 25% to 75% copper, 10% to 60% graphite, 5% to 25% barium fluoride, 0.1% to 5% boron nitride, 1% to 10% of at least one metal selected from the group consisting of tin, silver and lead and 1% to 5% coumarone indene resin.

12. An electrical contact brush adapted to operate efficiently at altitudes of at least 40,000 feet consisting of 25% to 75% copper, 10% to 60% graphite, 5% to 25% barium fluoride, 0.1% to 5% boron nitride and 1% to 5% coumarone indene resin.

13. An electrical contact brush adapted to operate efficiently at altitudes of at least 40,000 feet consisting of 25% to 75% copper, 10% to 60% graphite, 5% to 25% barium fluoride, and additive material consisting of 0.1% to 5% boron nitride, up to 5% coumarone indene resin

and up to 10% of at least one metal selected from the group consisting of lead, tin, and silver, said additive material comprising 0.5% to 15% by weight of said brush.

References Cited in the file of this patent

UNITED STATES PATENTS

|           |               |               |
|-----------|---------------|---------------|
| 1,121,960 | Whitney       | Dec. 22, 1914 |
| 1,299,846 | McCoy         | Apr. 8, 1919  |
| 2,156,803 | Cooper et al. | May 2, 1939   |
| 2,445,003 | Ramadanoff    | July 13, 1948 |
| 2,640,944 | Ramadanoff    | June 2, 1953  |
| 2,731,371 | Ramadanoff    | Jan. 17, 1956 |
| 2,739,254 | Moberly       | Mar. 20, 1956 |
| 2,844,544 | Ramadanoff    | July 22, 1958 |

FOREIGN PATENTS

|         |               |               |
|---------|---------------|---------------|
| 712,188 | Great Britain | July 21, 1954 |
|---------|---------------|---------------|